

Nov. 4, 1930.

W. W. McLaurin

1,780,793

COATED PAPER AND PROCESS OF MANUFACTURING SAME

Filed Nov. 6, 1926



INVENTOR  
William W. Lauri  
By  
John M. Cready,  
his ATTORNEY.

## UNITED STATES PATENT OFFICE

WILLIAM WALLACE McLAURIN, OF BROOKFIELD, MASSACHUSETTS

## COATED PAPER AND PROCESS OF MANUFACTURING SAME

Application filed November 6, 1926. Serial No. 146,630.

This invention relates to coated papers and to processes of manufacturing such papers.

In coating paper for high-grade printing or engraving a coating material is used which tends to harden and stiffen the sheet so that the finished paper will have a smooth hard surface. When such a paper is used for pamphlets, folders, or the like, where it is necessary to fold or crease the printed sheet, the paper breaks or cracks along the lines of folding. If it is attempted to modify the coating so as to produce a more pliable paper, the result is to impair the printing qualities of the sheet.

10 The present invention deals with the problem presented by these conditions, and it aims to overcome the objection above described. In other words, the invention aims to provide a coated paper for high-grade printing or engraving which can also be folded without breaking.

15 The nature of the invention will be readily understood from the following description when read in connection with the accompanying drawings, and the novel features will be particularly pointed out in the appended claims.

20 The single figure of the accompanying drawing is a diagrammatic perspective view illustrating a process of strip coating paper embodying the present invention.

According to the process illustrated in the drawing, a continuous strip S of paper is drawn from the supply roll 2 and travels over 25 a roll 3 having raised peripheral portions or rings 4 with which the paper is held in contact by means of another roll 5. The coating material is applied to certain areas or strips of the web S by the rings 4. A supply of the coating material is held in a tank 6, and a feed roll 7 which is partly submerged in the liquid coating material transfers it to an intermediate roller 8, usually covered with felt, which, in turn, delivers the material to the 30 rings 4 of the strip roll 3. This arrangement ensures the application of a limited and substantially uniform quantity of coating material to the paper. Strips of coating so applied are indicated at A. This coating 35 should be relatively "hard", that is, adapted

to impart to the finished sheet the hard, smooth surface which is desired for high-grade printing or engraving. Such coatings are well known to the trade so that no specific composition of a coating material need be given here. A typical coating compound may consist of clay, blanc fixe, satan white, and a suitable pulp color, together with a casein or glue sizing and water.

The paper next runs over a roll 9 and 40 into contact with another strip roll 10 having one or more annular portions or rings 12 to run in contact with the surface of the paper which has not already been coated by the strip roll 3. The rings 12 apply to 45 the uncoated sections of the paper a coating of material which gives to the paper a softer and more pliable finish than the coating previously applied. Such a compound, for example, may include the same ingredients 50 as the coating material above specified, and, in addition, certain softening materials, such as glycerine or glucose, or possibly fatty or oily constituents in limited quantities, as will be readily understood by those skilled in this 55 art. This material is mixed with water and the mixture fed to the strip roll 10 by a feed roll 14 and a transfer roll 15 in substantially 60 the same manner that the hard coating compound is fed to the strip roll 3. The strip 65 coatings applied by the roll 10 are indicated at B. From the latter roll the web of paper 70 travels over guide rolls 16 and 17 and is then wound up on a roll 18, suitable time being allowed in the travel of the strip to enable 75 the coating to dry. If desired, the web may be run over one or more heated rolls or drying 80 drums to hasten the drying operation.

In applying the coating materials to the 85 paper "doctors" or scrapers may be used on the feed rolls where a more accurate control of the thickness of the coating is required than can be obtained by the mechanism above described. Preferably the two coatings are 90 of substantially the same thickness so that 95 a level sheet is produced.

In performing the coating operation the width and shape of the areas coated are 100 predetermined with reference to the sheet to be printed so that the printing will be done on

the part A of the paper which has the harder coating, and the line or lines of fold will come on the strip B, which is softer and more pliable. In case it is desired to have the softer coated areas B extend both across as well as longitudinally of the sheet, the strip rolls 3 and 10 can be modified in shape to give this result, as will be evident to those familiar with paper coating operations.

10 The process above described produces a paper having dry and non-adhesive coatings, adjacent areas having quite different characteristics, the hard coated areas being admirably adapted for high-grade printing, while 15 the adjacent areas carrying the softer coating are especially adapted for folding and creasing.

It will be understood that the particular way in which the coatings are applied, the 20 widths and shape of the areas coated, and the like, will be determined by the use which is to be made of the paper. While, therefore, I have herein shown and described a typical arrangement for practicing the present invention, it will be understood that the process provided by this invention may be practiced in other ways without departing from the spirit or scope of the invention.

Having thus described my invention, what 30 I desire to claim as new is:

1. That improvement in processes of manufacturing coated papers which consists in applying a hard coating of non-adhesive material adapted to facilitate printing to a strip 35 of the area of said paper, and applying a softer coating of non-adhesive material to an adjoining strip of the surface of the paper.

2. That improvement in processes of strip coating paper which consists in applying a 40 coating of material adapted to produce a hard finish on the surface of the paper in spaced strips on said surface, and coating the intervening surface of the paper with a material adapted to produce a softer and more pliable finish, both of said coatings being 45 non-adhesive.

3. An article of the character described consisting of paper having adjacent portions of the surface thereof coated with different 50 compositions, the coating on one portion being adapted to render the paper hard and that on another portion making the paper more pliable, both of said coatings being non-adhesive.

55 4. An article of the character described comprising paper with a relatively hard coating thereon to facilitate printing, and a softer strip coating interrupting said hard coating and facilitating folding, both of said 60 coatings being non-adhesive.

5. An article of the character described comprising paper, the greater part of the surface on one side thereof being coated with a relatively hard non-adhesive material 65 adapted to facilitate printing, an adjacent

portion of said surface being coated with a softer non-adhesive material adapted to facilitate folding.

6. An article of the character described consisting of paper having on one face thereof adjacent strip coatings, one adapted to give the paper a hard finish and the other adapted to produce a more pliable finish, both of said coatings being non-adhesive.

WILLIAM WALLACE McLAURIN.

70

75

80

85

90

95

100

105

110

115

120

125

130